

## UNITED STATES PATENT OFFICE.

MICHAEL GEORGE KORSUNSKY, NOW BY JUDICIAL CHANGE OF NAME MICHAEL GEORGE CORSON, OF JACKSON HEIGHTS, NEW YORK, ASSIGNOR TO ELECTRO METALLURGICAL COMPANY, A CORPORATION OF WEST VIRGINIA.

## ALLOY FOR ELECTRICAL CONDUCTORS.

No Drawing.

Application filed December 9, 1924. Serial No. 754,857.

While copper is almost universally used for electrical conductors because of its high conductivity and resistance to corrosion, its relatively low tensile strength is often a 5 disadvantage, limiting the length of the spans of conductor which can be hung between supports. This is particularly important in the case of high-tension power-transmission lines where the supporting 10 structures are usually relatively expensive.

The tensile strength of copper can be increased by alloying it with various other metals and metalloids, but its conductivity is simultaneously diminished. Chromium is 15 probably the most effective addition to copper for increasing its tensile strength. Thus copper has a tensile strength of only about 35,000 pounds per square inch when annealed and only 54,000 to 56,000 pounds when 20 hard-drawn, while a copper-chromium alloy containing a small percentage of chromium has a tensile strength of 72,000 to 80,000 pounds as cold-rolled from the cast ingot. The conductivity of the copper-chromium 25 alloy as cold rolled from the ingot however, is only about 50%, Matthiesen standard, and it is therefore not comparable with copper as a material for electrical conductors.

If the cold-rolled alloy is heated for a 30 sufficient time at usual annealing temperatures its conductivity is considerably improved, but the annealed alloy has a tensile strength but little higher than that of annealed pure copper, so that it has no advantage over copper as a material for conductors.

The invention is a process whereby the conductivity of a strong copper alloy, such as a copper-chromium alloy, may be made 40 much higher than that exhibited by the cast alloy, without seriously impairing the tensile strength of the alloy. The invention also includes the product of this process and more particularly it includes alloys, for example copper-chromium alloys, having a conductivity in excess of 75%, M. S., and a tensile strength in excess of 70,000 pounds per square inch when in the form of wire of one-fourth inch diameter.

50 The process of the invention consists in annealing the alloy and so limiting the time and temperature of annealing that the above

mentioned result is attained. Temperatures as low as 400° C. may be used, but with such temperatures it requires two or three 55 hours to bring about the maximum increase in conductivity. Higher annealing temperatures make it possible greatly to reduce the annealing period, and indeed this period must be curtailed or the high tensile strength 60 characteristic of the cast alloy will be in a large measure lost. At about 700° C., the desired change in the alloy can be brought about in as little as five minutes in some cases. The above examples illustrating the 65 inverse relation between time and temperature and the preferred temperature range will enable those skilled in the art to practise the invention. The times will vary somewhat with the composition of the alloy, 70 but a few easily performed tests will suffice to fix the optimum conditions for a particular material.

My preferred alloy is copper containing 0.5% to 3.0% chromium. As the chromium 75 content is increased within the range indicated, the tensile strength of the alloy will increase, but the rate of increase falls off so that it will usually be uneconomical to use more than 3% of chromium.

I prefer also to incorporate into the alloy a deoxidizer such as silicon or phosphorus, which are to be regarded as equivalents for the purposes of this application. When 85 such deoxidizers are added to pure copper the conductivity of the copper falls off very rapidly with increasing percentage of the deoxidizer. For this reason, if the deoxidizers are added to pure copper to be used 90 for conductors, the quantity added must be very small, that remaining in the copper never exceeding about 0.01% in commercial practice. If, however, chromium is also present, the effect of the deoxidizers in reducing conductivity is very much less, and much higher percentages of the deoxidizer 95 may be used. This not only obviates manufacturing difficulties but it permits cleaner and sounder metals to be made. I prefer to add the deoxidizer in amount between 0.03% and 0.3%. About 0.2% of silicon or phosphorus gives good results. Unless sufficient deoxidizer is present to reduce any 100

cuprous oxid present, this will be reduced by the chromium, thereby destroying this latter valuable material and producing an oxidation product which is more difficult to 5 remove from the metal than the oxidation product of silicon or phosphorus.

In preparing alloy according to my invention, I first melt the copper under conditions minimizing oxidation. I then incorporate the deoxidizer in any usual or suitable way, the quantity added being generally not more than 0.3%. Under certain conditions considerably more than 0.3% of the deoxidizer may remain in the alloy without seriously decreasing its conductivity. Before the chromium is added, the temperature of the copper is raised to expedite alloying. A temperature of about 1275° C. gives good results, and it is usually undesirable to exceed 1350° C. since high temperatures promote oxidation of the chromium during alloying. The chromium should be added in pieces which are neither too small nor too large, since on the one hand too much oxidation takes place and on the other the alloying takes place too slowly. Pea-sized lumps of chromium are suitable. The bath should be stirred vigorously while the chromium is dissolving.

30 The foregoing is a preferred method of producing the alloy, but variations, such for example as adding the chromium as a pre-formed copper-chromium or other alloy, are permissible.

35 The metal may be cast and the ingots

more or less reduced in cross-section before annealing them in accordance with the invention, but the final drawing should follow the annealing in order that the finished wire or the like may have the high strength 40 which is characteristic of hard-drawn material. Alloys have been prepared in accordance with the invention which exhibit a conductivity of 80% coupled with a tensile strength of 72,000 to 80,000 pounds per 45 square inch.

I claim:

1. Process of treating an alloy containing 0.5% to 3.0% chromium with the balance substantially copper which comprises subjecting the alloy when it has substantially the tensile strength of the cast and hard-drawn material to a heat-treatment equivalent to annealing for two to three hours at 400° C., and then hard-drawing the annealed alloy into wire. 50

2. Process of treating an alloy containing 0.5% to 3.0% of chromium with the balance substantially copper which comprises subjecting such alloy, in a condition wherein 60 it has a high tensile strength, to an annealing operation in the temperature range 400° C. to 700° C. and of such regulated duration that the conductivity of the cold alloy is increased to at least 75% M. S. and the 65 tensile strength is not reduced below 70,000 pounds per square inch.

In testimony whereof, I affix my signature.

MICHAEL GEORGE KORSUNSKY.